

1

3,575,735  
OXIDATION PROTECTIVE COATINGS FOR  
VANADIUM ALLOYS

Dean B. Lawthers, Pittsburgh, Pa., assignor to the United States of America as represented by the Secretary of the Navy  
No Drawing. Filed Oct. 9, 1968, Ser. No. 766,309  
Int. Cl. C23c 9/00

U.S. Cl. 148—6

2 Claims

### ABSTRACT OF THE DISCLOSURE

A slurry for coating vanadium base alloys to provide oxidation protection comprising a metal of either silver, tin, or copper, silicon, and a carrier such as nitrocellulose lacquer, to which also may be added aluminum and columbium.

### BACKGROUND OF THE INVENTION

The present invention relates to vanadium alloys and more particularly to a slurry coating for vanadium based alloys for providing resistance to oxidation.

Vanadium based alloys have a promising future, particularly in aerospace applications, as these alloys have low density, good ductility, and weldability. However, oxidation has been a serious problem as the formation of molten vanadium pentoxide upon exposure to air at the relatively low temperature of 1250 degrees F. results in catastrophic failure. In order to overcome this weakness, various oxidation protection systems have been studied for vanadium alloys. One promising system involves a pack siliconizing treatment that leads to the formation of a surface compound with the base metal, resembling the processes used to protect columbium and molybdenum.

### SUMMARY OF THE INVENTION

The present invention relates to a slurry coating for vanadium based alloys and has several advantages. First, the slurry coating of the present invention eliminates various inherent disadvantages of pack siliconizing such as warpage and nonuniformity of coatings. Second the slurry coating of the present invention can be used to patch or repair defects in coatings formed by the pack siliconizing method.

In the present invention, a slurry is made by adding silicon and a metal such as silver, tin, or copper to a nitrocellulose lacquer, which decomposes during heat treatment. The metal and silicon is diffused with the base alloy in vacuum or under an argon atmosphere.

### DESCRIPTION OF THE PREFERRED EMBODIMENTS

The surface of a specimen to be given a slurry coating is first prepared by grit blasting, followed by pickling in a dilute acid bath. The specimen is then rinsed in acetone and dipped in the slurry composition. The slurry composition might be composed of silicon and a metal, such as silver, tin, and copper which are suspended in a nitrocellulose lacquer. Commercially available nitrocellulose lacquer can be used but it should be clear and unpigmented. Collodion is one type of commercial lacquer which can be used. The lacquer constitutes the liquid vehicle for the dispersal of the particulate silver, tin, or copper, and the silicon during coating. The lacquer must have an adequate "green" strength to hold the coating in place after being air cured and during heat treating. The lacquer decomposes during heating, leaving only a small amount of residue which does not adversely affect the final coating.

2

A weight percentage of between 60 and 80 percent silver to between 20 and 40 percent silicon is considered to provide optimum processing conditions and this range tends to insure a sufficient supply of each material throughout the coating to produce a uniform coating. In this connection, the silver is not a constituent of the final silicide coating, but rather the vehicle in which the silicon may migrate to the surface of the vanadium alloy to react with the vanadium to produce  $VS_2$ . The silver is vaporized off during the heat treatment. Both tin and copper have been shown to be effective substitutes for silver. The ratio of lacquer to powdered ingredients is not critical and will depend upon the means employed in applying the coating to the specimen. For example, a ratio of about 5 parts powder to 1 part lacquer (by weight) might be employed for a dip coating and a ratio of about 4 parts powder to 1 part lacquer might be employed for a spray coating.

The following examples exemplify the present invention:

#### EXAMPLE 1

A slurry was made with the following percentages of ingredients, by weight:

|                        |       |
|------------------------|-------|
| Silver                 | 56.25 |
| Silicon                | 18.75 |
| Nitrocellulose lacquer | 25.00 |

A test specimen of 60 percent vanadium, 39 percent columbium and 1 percent titanium was grit blasted and then pickled in  $25\text{NHO}_3$ — $5\text{HF}$ — $70\text{H}_2\text{O}$ , and then rinsed in acetone. The test specimen was then dipped in the slurry and allowed to air dry. The test specimen was then given a diffusion treatment in a stainless steel muffle in a tube type furnace. A vacuum was first pulled on the muffle and then an argon flow was started. The diffusion treatment was conducted at a temperature of about 1800 degrees F. for a period of four hours under a dynamic argon atmosphere. The resultant coating was between 0.001 and 0.002 inch in thickness with the desired silicide layer being about 0.0005 inch. In an oxidation test, the test specimen was heated to a temperature of 2200 degrees F. and failure resulted in about 1 hour.

#### EXAMPLE 2

A slurry was made with the following percentages of ingredients, by weight:

|                        |       |
|------------------------|-------|
| Tin                    | 56.25 |
| Silicon                | 18.75 |
| Nitrocellulose lacquer | 25.00 |

A test specimen was cleaned, dipped, and diffused as in Example 1. In an oxidation test, the test specimen was heated to a temperature of 2200 degrees F. and failure resulted in about 1 hour.

#### EXAMPLE 3

A slurry was made with the following percentages of ingredients, by weight:

|                        |    |
|------------------------|----|
| Copper                 | 60 |
| Silicon                | 15 |
| Nitrocellulose lacquer | 25 |

A test specimen was cleaned, dipped, and diffused as in Example 1. In an oxidation test, the test specimen was heated to a temperature of 2200 degrees F. and failure resulted in about 1 hour.

**3**  
**EXAMPLE 4**

A slurry was made with the following percentages of ingredients, by weight:

|                              |      |
|------------------------------|------|
| Silver -----                 | 53.5 |
| Silicon -----                | 17.9 |
| Sodium fluoride -----        | 3.6  |
| Nitrocellulose lacquer ----- | 25.0 |

A test specimen was cleaned as in Example 1 and then dipped in the slurry. After air drying, the test specimen was dipped a second time and the resultant coating was between 0.002 and 0.003 inch in thickness with the desired silicide coating being about 0.001. Sodium fluoride was added as an activator and flux. The test specimen was diffused as in Example 1. In an oxidation test, the test specimen was heated to a temperature of 2200 degrees F. and failure resulted in about 10 hours.

**EXAMPLE 5**

A slurry was made with the following percentages of ingredients, by weight:

|                              |      |
|------------------------------|------|
| Tin -----                    | 53.5 |
| Silicon -----                | 17.9 |
| Sodium fluoride -----        | 3.6  |
| Nitrocellulose lacquer ----- | 25.0 |

A test specimen was cleaned, dipped, and diffused as in Example 4, that is, it was given a double-dipped treatment. In an oxidation test, the test specimen was heated to a temperature of 2200 degrees F. and failure resulted in about 10 hours.

**EXAMPLE 6**

A slurry was made with the following percentages of ingredients, by weight:

|                              |      |
|------------------------------|------|
| Copper -----                 | 57.2 |
| Silicon -----                | 14.2 |
| Sodium fluoride -----        | 3.6  |
| Nitrocellulose lacquer ----- | 25.0 |

A test specimen was cleaned, dipped, and diffused as in Example 4. In an oxidation test, the test specimen was heated to a temperature of 2200 degrees F. and failure resulted in about 10 hours.

**EXAMPLE 7**

A slurry was made with the following percentages of ingredients, by weight:

|                              |       |    |
|------------------------------|-------|----|
| Tin -----                    | 48.75 | 50 |
| Aluminum -----               | 18.75 |    |
| Columbium -----              | 5.63  |    |
| Silicon -----                | 1.87  |    |
| Nitrocellulose lacquer ----- | 25.00 |    |

The test specimen was cleaned, double-dipped, and diffused as in Example 4. In an oxidation test, the test specimen was heated to a temperature of 2200 degrees F. and lasted longer than 10 hours before failure.

**4**  
**EXAMPLE 8**

A slurry was made with the following percentages of ingredients, by weight:

|                              |      |
|------------------------------|------|
| Tin -----                    | 51.4 |
| Aluminum -----               | 15.0 |
| Silicon -----                | 8.6  |
| Nitrocellulose lacquer ----- | 25.0 |

The test specimen was cleaned, double-dipped in the slurry and diffused as in Example 4. In an oxidation test, the test specimen was heated to a temperature of 2200 degrees F. and failure resulted in 30 hours.

In comparing the above-examples, the test specimens that were given a double coating had a substantially increased oxidation life at a temperature of 2200 degrees F. For example, the specimens that were given a single dip coating failed in about one hour, while a second coating increased the oxidation life to 10 hours or longer.

Obviously many modifications and variations of the present invention are possible in the light of the above teachings. For example, satisfactory coatings have been diffused at a temperature range between 1800 and 2000 degrees F. for a period between 1 and 4 hours. It is therefore to be understood, that within the scope of the appended claims, the invention may be practiced otherwise than as specifically described.

1. A high temperature oxidation resistance composition of matter for coating vanadium based alloys consisting, by weight, of
  - between 48 and 68 percent of a metal selected from the group consisting of silver, copper, and tin,
  - between 1.5 and 20 percent silicon,
  - between 15 and 25 percent aluminum, and
  - between 15 and 25 percent nitrocellulose lacquer.
2. A method for applying an oxidation resistance coating to vanadium based alloys comprising:
  - coating a member formed of said vanadium base metal by dipping in a slurry consisting, by weight, of between 48 and 68 percent of a metal selected from the group consisting of silver, copper, and tin, between 1.5 and 20 percent silicon, between 15 and 25 percent aluminum, and between 15 and 25 percent nitrocellulose lacquer, and
  - then diffusing said coating by heating said member in an inert atmosphere at a temperature between 1800 and 2000 degrees F. for a period of 1 to 4 hours.

**References Cited**

**UNITED STATES PATENTS**

2,883,282 4/1959 Wainer ----- 75—174  
3,166,409 1/1965 Hubbard ----- 75—134

ALFRED L. LEAVITT, Primary Examiner

C. WESTON, Assistant Examiner

U.S. CL. X.R.

29—197, 198; 106—1; 117—2, 46, 131, 135.1